

## UNITED STATES PATENT OFFICE

2,426,416

## ELECTROPLATING NICKEL

Ernest W. Schweikher, Cleveland Heights, Ohio,  
assignor to E. I. du Pont de Nemours & Company, Wilmington, Del., a corporation of Delaware

No Drawing. Application June 10, 1941,  
Serial No. 397,383

6 Claims. (Cl. 204—49)

1

This invention relates to the electrodeposition of nickel and is more particularly directed to nickel plating compositions, nickel plating baths, and nickel plating processes wherein there is employed a composition as follows:

|                       | Grams per liter |
|-----------------------|-----------------|
| Nickel chloride       | 225 to 275      |
| Nickel sulfate        | 15 to 60        |
| Boric acid            | 45 to 60        |
| Metasulfobenzaldehyde | 4 to 10         |

It has previously been proposed to use a sulfobenzaldehyde as an addition agent for nickel plating. It has also been proposed recently to use nickel sulfate in nickel chloride baths the ratio of chloride anion to sulfate anion falling within the range from 5:1 to 20:1.

It is an object of this invention to provide compositions, baths, and processes by the use of which there may be obtained bright nickel deposits of excellent character. It is a further object to provide compositions, baths, and processes which require a minimum of maintenance and which over considerable periods of time will consistently produce deposits of excellent and uniform character. It is a still further object to provide nickel plating compositions, baths, and processes by the use of which there may be obtained nickel deposits which are brilliant and ductile even over long periods of operation. Still further objects of this invention will become apparent hereinafter.

The foregoing and other objects are attained by the use of a bath composition as follows:

|                       |                 |            |
|-----------------------|-----------------|------------|
| Nickel chloride       | grams per liter | 225 to 275 |
| Nickel sulfate        | do              | 15 to 60   |
| Boric acid            | do              | 45 to 60   |
| Metasulfobenzaldehyde | do              | 4 to 10    |
| pH                    |                 | 2.0 to 4.0 |

I have found that metasulfobenzaldehyde in this particular bath with boric acid present in amounts from about 45 to 60 grams per liter as shown yields particularly excellent results over long periods of time with a very minimum of maintenance. Each component in the proportions recited cooperates with the others to produce the unexpected results of the invention.

A preferred illustrative bath of the present invention is described in the following example:

2

## Example

A nickel plating bath was made up as follows:

|                                                               |                 |        |
|---------------------------------------------------------------|-----------------|--------|
| Nickel chloride ( $\text{NiCl}_2 \cdot 6\text{H}_2\text{O}$ ) | grams per liter | 250    |
| Nickel sulfate ( $\text{NiSO}_4 \cdot 7\text{H}_2\text{O}$ )  | do              | 15     |
| Boric acid ( $\text{H}_3\text{BO}_3$ )                        | do              | 50     |
| Metasulfobenzaldehyde                                         | do              | 4      |
| pH                                                            |                 | 3.5    |
| Temperature                                                   |                 | 50° C. |

Brilliant nickel deposits were made from the bath of this example at a current density of about 35 amperes per square foot and a number of articles which had previously been copper plated were given pit-free, ductile deposits which without further buffing or polishing served admirably as a base surface for chromium plating.

The temperature of the baths of this invention during operation may vary but it will be preferred to use temperatures between about 45 and 55° C. Deposits of desirable character will ordinarily be produced at current densities from about 5 to 125 amperes per square foot.

In the use of the bath of this example there was employed electrolytic cathode nickel as anodes. It is one of the advantages of this type of bath that cathode nickel may be used as anode without any special treatment.

While reference is made herein to the addition of metasulfobenzaldehyde, it will be understood that the addition agents may be added to a plating bath in the form of various salts. It may, for instance, be added to the bath in the form of a sodium, potassium, ammonium, or nickel salt. Whether or not the sulfobenzaldehyde is present in the bath as a salt or as a free acid will depend upon the pH of the bath and consequently for the purposes of this invention either the acid or a suitable salt may be used interchangeably. As a matter of fact, the metasulfobenzaldehyde was added in the composition of the above example as the nickel salt.

The baths of this invention may be modified by the inclusion of additions known to benefit electroplating baths. The addition agents of the Lutz-Westbrook Patent 1,818,229 may be used and there may similarly be used the addition agents of Schlotter 1,972,693, Waite 2,112,818, Flett 2,195,409, Pine 2,029,386 and 2,029,387, Lynn,

Harshaw, and Long 2,198,267 and 2,198,268, and Harshaw and Long 2,125,229. While such additions or mixtures of such addition agents may be made to the baths of this invention it will ordinarily be found most desirable not to use other bath-improving agents and according to the preferred practices of this invention there is employed an electroplating bath consisting essentially of the following at the proportions shown:

Nickel chloride \_\_\_\_\_ grams per liter 225 to 275  
 Nickel sulfate \_\_\_\_\_ do 15 to 60  
 Boric acid \_\_\_\_\_ do 45 to 60  
 Metasulfobenzaldehyde \_\_\_\_\_ do 4 to 10  
 pH \_\_\_\_\_ 2.0 to 4.0  
 Temperature \_\_\_\_\_ 50° C.

Plating compositions as offered to the trade may conveniently contain all of the ingredients tabulated and in referring to a plating composition it will be understood that the composition may be dry or it may be a concentrated solution suitable for use upon dilution as well as the dilute solution ready for use as an electroplating bath. If preferred, the individual constituents may be supplied to an electroplater so that the composition may be made up at the place of use by dissolving the various ingredients simultaneously or individually in water.

While I have shown certain compositions, baths, and processes, it will be understood that one skilled in the art may readily devise numerous similar compositions, baths, and processes without departing from the spirit of the invention.

I claim:

1. An aqueous nickel plating bath comprising:

Nickel chloride \_\_\_\_\_ Grams per liter 225 to 275  
 Nickel sulfate \_\_\_\_\_ 15 to 60  
 Boric acid \_\_\_\_\_ 45 to 60  
 Metasulfobenzaldehyde \_\_\_\_\_ 4 to 10

2. An aqueous nickel plating bath comprising substantially:

Nickel chloride (NiCl<sub>2</sub>·6H<sub>2</sub>O) \_\_\_\_\_ Grams per liter 250  
 Nickel sulfate (NiSO<sub>4</sub>·7H<sub>2</sub>O) \_\_\_\_\_ 15  
 Boric acid (H<sub>3</sub>BO<sub>3</sub>) \_\_\_\_\_ 50  
 Metasulfobenzaldehyde \_\_\_\_\_ 4

3. In a process for the electrodeposition of

nickel, the step comprising effecting electrodeposition from an aqueous nickel plating bath comprising:

5. Nickel chloride \_\_\_\_\_ Grams per liter 225 to 275  
 Nickel sulfate \_\_\_\_\_ 15 to 60  
 Boric acid \_\_\_\_\_ 45 to 60  
 Metasulfobenzaldehyde \_\_\_\_\_ 4 to 10

6. In a process for the electrodeposition of nickel, the step comprising effecting electrodeposition from an aqueous nickel plating bath comprising substantially:

15 Nickel chloride (NiCl<sub>2</sub>·6H<sub>2</sub>O) \_\_\_\_\_ Grams per liter 250  
 Nickel sulfate \_\_\_\_\_ 15  
 Boric acid \_\_\_\_\_ 50  
 Metasulfobenzaldehyde \_\_\_\_\_ 4

20 7. A nickel plating composition which upon addition of water will yield a solution of the following in the indicated proportions:

Grams per liter  
 Nickel chloride \_\_\_\_\_ 225 to 275  
 Nickel sulfate \_\_\_\_\_ 15 to 60  
 25 Boric acid \_\_\_\_\_ 45 to 60  
 Metasulfobenzaldehyde \_\_\_\_\_ 4 to 10

30 8. A nickel plating composition which upon addition of water will yield a solution of the following in the indicated proportions:

Grams per liter  
 Nickel chloride (NiCl<sub>2</sub>·6H<sub>2</sub>O) \_\_\_\_\_ 250  
 Nickel sulfate (NiSO<sub>4</sub>·7H<sub>2</sub>O) \_\_\_\_\_ 15  
 Boric acid (H<sub>3</sub>BO<sub>3</sub>) \_\_\_\_\_ 50  
 35 Metasulfobenzaldehyde \_\_\_\_\_ 4

ERNEST W. SCHWEIKHER.

#### REFERENCES CITED

40 40 The following references are of record in the file of this patent:

#### UNITED STATES PATENTS

| Number    | Name        | Date          |
|-----------|-------------|---------------|
| 2,191,813 | Brown       | Feb. 27, 1940 |
| 2,198,267 | Lind et al. | Apr. 23, 1940 |

#### OTHER REFERENCES

Physical Review, Second Series (1925), volume 26, pages 390 and 396.